

## UNITED STATES PATENT OFFICE

2,103,999

DISINFECTIVE AND ANTISEPTIC COMPOUND  
FOR THE TREATMENT OF ULCERS, SORES,  
AND THE LIKE

John H. Müller, Secane, Pa.; Anna L. Müller and  
Provident Trust Co., executors of said John H.  
Müller, deceased, assignors to Silver Oxide  
Products Company, Incorporated, a corpora-  
tion of Pennsylvania

No Drawing. Application May 25, 1936,  
Serial No. 81,645

6 Claims. (Cl. 167—72)

This application for Letters Patent is, in part, a continuation of my pending application for Letters Patent, entitled "Disinfective and antiseptic compound for the treatment of ulcers, sores and the like", filed September 27, 1933, which has received the Serial Number 691,246, and my invention relates to the preparation of a fluid or semi-fluid compound having a disinfective and antiseptic effect when applied to the treatment of ulcers, sores, abrasions, various skin eruptions or the like or to any more or less infected surfaces of a human or animal body whether such surfaces exist in internal or external portions of the body and which can be applied without injury to healthy cellular tissue and my invention consists in a colloidal suspension and distribution of silver oxide in a non-reactive and inert fluid or semi-fluid vehicle and particularly, and for I believe, the best results, in a colloidal suspension of silver oxide in one of the or a mixture of aliphatic hydrocarbons of the paraffin series comprehended within the general formula  $C_nH_{2n+2}$ . This class of hydrocarbons is, to a marked degree, nonreactive with colloidal silver oxide. The inactivity of the paraffin hydrocarbons toward silver oxide constitutes an important factor in my new remedial compound because this very active oxide should exist in the preparation as such without any chemical reaction with the fluid or semi-fluid carrier. It is a matter of chemical knowledge that all or practically all vehicles of an organic nature cannot remain in contact with silver oxide without more or less rapid reduction of the oxide to metal or formation of complex silver compounds and hence such mixtures cannot be construed as mixtures of silver oxide of known composition.

In referring to the condition of the silver oxide as colloidal, I mean that the particle size of the oxide distributed through the inert vehicle should predominantly and preferably entirely be of dimensions less than that of a micron and in practice I have found it desirable that the particles should predominantly be of dimensions approximating one-half to three-tenths or less of a micron. This fine division of the silver oxide content of the compound is important both because it brings about a great mobility of the silver oxide particles in the fluid or semi-fluid vehicle so that, on application to a surface the contained silver oxide particles come into contact with the treated surface very shortly after application, and, also because this fine division of the silver oxide results in giving to each particle a relatively enormous surface in relation to

its mass so that, on coming into contact with the watery fluids of the body, the small particle of silver oxide is rapidly converted into a solution of silver hydroxide which, while highly efficient as a disinfectant, acts as such in a quite different way from that of common silver oxide applied in more ponderable particles in that it has no tendency to cauterize and injure healthy tissue and is not liable to bring about any permanent stains in the body to which it is applied, such silver as is evolved from my compound in the deoxidation of the silver oxide passing off with the wastes of the body.

It is also true, I have found, that the exceedingly small particle size of the colloidal silver oxide enables it to pass through the normal skin of man or animal, or through the pores promptly reaching the more watery tissue and entering the blood stream, no doubt as a hydroxide or other form of ionic silver solution and thus reaching infected regions of the body not ordinarily accessible by superficial application of a medicinal compound.

My new compound can be conveniently manufactured by precipitating silver oxide from an aqueous solution of silver nitrate by addition of an excess of sodium hydroxide. The precipitated oxide is filtered and washed upon suction filters with distilled water until free from other products of the reaction. The residual mass of finely divided silver oxide is then freed as far as possible from water by continued suction and is then dehydrated in special ovens protected from dust or other reducing influences. It is then mixed in known ratio by weight with the non-reactive hydrocarbon vehicle. This mixture is then passed through a colloid mill and is further subjected to dispersion in a pebble mill until required particle size is obtained. This, when carried out to a sufficient extent, produces a colloidal suspension of known silver oxide content which can be subsequently diluted with a non-reactive hydrocarbon or hydrocarbon mixtures, (paraffins), of any desired consistency so as to give a final product of any required fluidity and known content of colloidal silver oxide. It has been found in practice that mixtures containing five percent of silver oxide or as little as one half of one percent of the same are adapted to common use but any desired concentration of the colloidal silver oxide can be prepared at the discretion of the physician in the treatment of special cases. I have found in practice that to produce a proper colloidal comminution of the silver oxide so that it will contain particles of

half a micron, average size, weeks of grinding are required when a pebble mill is used.

My new compound is of such a character that it remains substantially without change of active constituent of colloidal silver oxide until the mixture is applied to the tissues under treatment.

When such contact is established, as by distributing the compound over the surface to be treated, the compound acts as a reservoir from which the colloidal particles of silver oxide progressively contact with the surface until the fluid or semi-fluid vehicle is practically denuded of the suspended colloidal silver oxide particles and the silver oxide particles coming thus progressively

10 in contact with the treated surface pass into the normal skin or its pores and into contact with the more watery cellular tissue lying beneath it or adjacent to it into direct contact with cellular tissue not protected by the normal skin and/or absorbed into such cellular tissue and thence pass

15 into the blood stream without any caustic action upon the surfaces of tissues treated, such as would tend to injure normal tissue and presumably as a silver hydroxide solution, the effect being to act

20 as a disinfectant of not only the immediate surface treated but also adjacent portions of the body not directly accessible, this being accomplished without such liability of bringing about deposits of silver in the treated surface or elsewhere forming permanent discolorizations.

25 My new compound, which is a mixture of colloidal silver oxide in an inactive vehicle, takes on a mildly alkaline nature when brought in contact with the water invariably present in living tissues. In this way silver oxide mixture is pur-

30 posey used as a reservoir for production of silver hydroxide, a mild alkaline oxidant which is harm-

35 less to normal cellular structures and comparable in alkalinity with blood plasma itself.

40 It will be understood that the essential feature of my new medicinal compound lies in the com-

45 bination of a colloidal subdivision and distribution of the silver oxide with the inert vehicle which minimizes any tendency to the formation of aggregates of the oxide particles so that, on application, the colloidal particles of silver oxide come progressively into contact with the tissues of the body to which it is applied and are available for rapid absorption thereby, presumably as a

45 silver hydroxide solution, and certainly without any such cauterizing effect upon the tissues

treated as is often brought about by the application of the common silver oxide in more ponderant states of subdivision and without danger of bringing about a staining of the skin caused by silver in the reduced condition, such as has been liable to occur on the application of other silver compounds.

Having now described my invention, what I claim as new and desire to secure by Letters Patent is:

10 1. The method of preparing a form of silver oxide which will dissolve and form the hydroxide without undergoing substantial reduction to form metallic silver when brought into contact with the human skin, which comprises precipitating 15 silver oxide in an aqueous vehicle, drying such precipitate and then mechanically grinding such oxide, while protected against moisture by an inert, oily, anhydrous vehicle until it has an average particle size of less than one micron diameter. 20

2. A method as specified in claim 1, in which the grinding is continued until the average particle size of the silver oxide is less than one-half of a micron.

25 3. Anhydrous colloidal silver oxide in the form of particles of an average diameter of less than one micron and small enough so that when a thin film of a dispersion of such particles in an inert, oily, anhydrous vehicle is brought into contact with a moist body such as the human skin, the silver particles will migrate to the contact boundary and pass into solution as silver hydroxide without leaving any substantial surface marking of reduced silver. 30

4. Silver oxide as specified in claim 3, in which the average particle size is less than one-half a micron.

35 5. A dispersion in an inert, anhydrous, oily vehicle of silver oxide in the form of colloidal particles of average diameter of less than one 40 micron and small enough so that when a thin film of such dispersion is brought into contact with a moist body such as a human skin, the silver particles will migrate to the contact boundary and pass into solution as silver hydroxide without leaving any substantial surface marking of reduced silver. 45

6. A dispersion as specified in claim 5 in which the inert vehicle is an aliphatic hydrocarbon of the paraffin series.

50 JOHN H. MÜLLER.